

May 12, 1959

J. L. SHELDON

2,886,730

APERTURE MASK COATING TO PREVENT CATHODE POISONING

Filed Feb. 25, 1957



Fig. 1



Fig. 2



Fig. 3

INVENTOR.  
JOHN L. SHELDON

BY  
Clarence R. Patty, Jr.

ATTORNEY

1

2,886,730

## APERTURE MASK COATING TO PREVENT CATHODE POISONING

John L. Sheldon, Corning, N.Y., assignor to Corning Glass Works, Corning, N.Y., a corporation of New York

Application February 25, 1957, Serial No. 642,074

3 Claims. (Cl. 313—86)

This invention relates to an improved perforate mask for assembly in a cathode ray tube of the type used in multicolor television receivers and to a cathode ray tube embodying such mask.

Certain types of multicolor television systems operate on the general principle of emitting a stream of electrons from one or more electron guns mounted in the neck of a cathode ray tube and directing such stream of electrons through a perforate mask onto a viewing screen composed essentially of a phosphor pattern deposited on a face plate or panel forming the opposite end of the tube. The perforate mask, for example the present tube component commonly referred to as a shadow or aperture mask, is positioned transversely of the electron path intermediate the electron gun and screen to intercept all electrons striking the mask and thereby form a plurality of electron beams passing through the apertures or perforations in the mask to the pattern of phosphors on the face of the tube. Multicolor television systems of this sort are described in detail in the patent literature, such as United States Patent #2,625,734 to Harold F. Law.

The apertures in such a mask are small and closely spaced, and must be formed with an extreme degree of accuracy to produce a clear, well-defined picture. Thus specifications of a typical mask call for apertures 10 mils in diameter and uniformly spaced 28 mils center to center and a mask thickness of 55 mils, with the aperture dimensions being held within a tolerance of  $\pm 0.5$  mil. The inherent difficulties in producing and handling such a mask are quite readily apparent. Furthermore it is frequently necessary to sag or otherwise form such a mask to a definite curvature.

Etched metal masks have been proposed, but their use requires a great deal of care to avoid warpage, bending, or other physical damage during production and subsequent handling. It has been recognized that a mask composed of a ceramic material such as glass should be highly desirable, but, until discovery of the chemical method of machining glass described in United States Patent #2,628,160 issued to S. D. Stookey, no satisfactory method existed for producing such masks. It was naturally assumed that, if a mask of glass or other ceramic could be satisfactorily produced, its use in a tube should present no particular problem since glass is used in construction of the tube envelope itself and other ceramics are widely used in electronic tubes.

Once glass masks were successfully made by the Stookey method, it was quite unexpectedly found that tubes embodying such masks in their assembly tended to fail shortly after being placed on life test. Extensive investigations into these tube failures indicated that the failure was due to a foreign material poisoning the cathode of the electron gun during its operation and that this foreign material was in some manner coming from the glass mask. It is then a primary purpose of the present invention to provide chemically perforated glass masks free from such prior deficiencies and capable of being used in cathode ray tubes for absorption of electrons.

2

By way of illustration the present invention is described with reference to the accompanying drawing in which,

Fig. 1 is a schematic representation, largely in section, of a cathode ray tube and,

5 Fig. 2 is an enlarged fragmentary view in section of a perforate mask in accordance with the invention and,

Fig. 3 is an enlarged fragmentary view in section, similar to Fig. 2, illustrating a modification of the invention.

In accordance with the present invention, satisfactory 10 glass aperture masks are produced by providing the electron intercepting surface of a chemically perforated glass mask with a coating composed of at least one layer of metal. By "electron intercepting surface" I mean the glass surface facing, and therefore exposed to, the electron 15 emission gun and hence to the stream of electrons emitted therefrom.

The cathode ray tube, schematically represented in Fig. 1 and designated by the numeral 10, has an electron gun 12 mounted in the tube neck 14 and a viewing screen 16 20 composed of a phosphor coating 18, of suitable composition and pattern for multicolor televising, applied to the inside surface of transparent face plate or panel 20 which forms the opposite, enlarged end of the tube. The phosphor coating is applied in any known manner in a dot, 25 stripe or other type of pattern suitable for the purpose. Mounted intermediate electron gun 12 and screen 16, by any suitable conventional means not specifically shown, is perforate glass mask 22, having a metal coating 24 on the side of the mask facing gun 12, that is the electron 30 intercepting surface of the mask.

In Fig. 2 a fragment of mask 22 is shown greatly exaggerated to better illustrate chemically perforated apertures 26 which are too small and too numerous to be satisfactorily shown in a full view such as Fig. 1, and to 35 better illustrate, as well, metal coating 24. In accordance with the exemplary mask specifications referred to earlier, the diameter of apertures 26 is 10 mils and they are spaced 28 mils apart center to center. For purposes of illustration mask 22 is shown flat and apertures 26, as shown, are 40 formed normal to the electron intercepting surface. As a practical matter mask 22 will frequently have imparted to it a definite curvature and apertures 26 may be formed at angles up to  $25^\circ$  or so from normal depending on the 45 location and geometry of the tube components. The angle of each aperture will be such as to provide alignment of electron gun, apertures and screen elements for proper screen scanning.

In a preferred embodiment of my invention the electron intercepting surface of mask 22 is coated with a layer 50 of metal 24 of sufficient thickness that electrons emitted by gun 12 are absorbed by the metal and do not penetrate to the glass to any appreciable extent. The exact effect of electron bombardment on chemically perforated glass has not been positively ascertained. It is my belief 55 however that absorption of electrons by this particular type of glass results in a reaction within the glass accompanied by evolution of a gas which poisons the electron gun cathode, and there is experimental evidence indicating that the offending gas is oxygen. In any event it has 60 been found that, if the glass is shielded by an absorbing layer of metal, poisoning of the cathode is either eliminated or so minimized that normal tube life can be expected.

Various methods of applying metal to glass surfaces are 65 available and may be used in coating glass masks. The process of thermal evaporation is a convenient one since it is well developed commercially to provide an adherent metal coating of controlled and adequate thickness on a glass surface. When this coating method is employed I 70 prefer aluminum as the coating metal since it is satisfactory for electron interception, and thermal evaporation of it is an established and well-understood process in the

manufacture of cathode ray tubes. However other inert metals such as iron, nickel, and alloys of these metals may also be satisfactorily used and in some instances may even be preferable because of greater density.

Thermally evaporated aluminum films heretofore employed in cathode ray tube production have been deposited as a conducting layer in conjunction with the phosphor screen on the tube face plate. Such a conducting film extends to an electrical contact or terminal through the tube wall and serves as a metallic conductor to drain electrons from the screen and return them to the power supply. The thickness of such conducting aluminum films is generally on the order of 3000 to 5000 Angstrom units and is minimized to avoid producing any substantial absorption effect on the stream of electrons directed at the screen.

The thickness of metal required on the glass mask for electron absorption purposes is of considerably greater magnitude and depends primarily on the voltage drop from the electron gun to the tube screen, that is the velocity of the electrons to be intercepted, and on the effective density of the metal coating employed, which in turn depends on the particular metal used. By way of specific illustrative example, a glass mask, designed for use in a cathode ray tube to operate at a rated voltage of 25 kilovolts, was provided with an aluminum film having a thickness of 75,000 Angstrom units and the resulting tube found to perform satisfactorily during a life test of 1000 hours which is considered to indicate a satisfactory tube for commercial use. On the basis of theory an aluminum coating 55,000 Angstrom units in thickness should be adequate but in order to provide an adequate safety factor I prefer to employ a thickness of 75,000 to 125,000 Angstrom units. While greater thicknesses could of course be used, they appear to be unnecessary and uneconomical.

The thickness required will vary directly with the square of the voltage and inversely with density. Thus, if a lower operating voltage than 25 kilovolts were being used, the minimum thickness might be correspondingly reduced. Likewise with another metal having, for example, an effective density, as deposited, three times that of aluminum, the minimum thickness would be one third or about 25,000 Angstrom units.

An alternative form of the invention is illustrated in Fig. 3 wherein the electron intercepting surface of mask 22 is coated with two layers of metal 28 and 30. Metal layer 28 is relatively thin and in direct adherent contact with the surface of mask 22. The metal employed should be a very chemically active metal, such as barium, which will act in the manner of a "getter" to immediately react with any oxygen or other cathode poisoning material evolved from the glass as a result of electron absorption. Other active metals, or getters, such as magnesium might also be employed, and any metal capable of spontaneously reacting with or absorbing cathode poisoning agents such as oxygen are contemplated for the present purpose. Metal layer 30, also relatively thin, is composed of an

inactive or inert metal and serves to protect the active metal layer 28 from atmospheric gases with which the mask is in contact while the tube is being assembled and prior to the conventional bakeout process. Metal layer 5 30, then, may be composed of an inert metal such as aluminum, iron, nickel, or the like. The duo-layered metal coating 28-30 is preferably applied to mask 22 by means of a two-step thermal evaporation process carried out in a suitable vacuum chamber. Thus, for example mask 22 might be mounted in a conventional thermal evaporation apparatus with suitable amounts of metallic barium and metallic aluminum positioned for thermal evaporation. The barium would be first deposited on the mask surface followed by deposition of a protective aluminum coating.

While the overall thickness of the double metal coating required in this embodiment of the invention will vary somewhat depending on tube operating conditions, it will, generally speak, be much thinner than an electron 20 absorbing type of film such as described earlier. The duo-layer coating is of course not intended to absorb electrons. The barium portion of the film then need be only of sufficient thickness to react with gases evolved, and the inert protective film need only be of sufficient 25 thickness to provide an effective barrier between the active metal and the atmosphere. It may correspond to the conducting films heretofore applied over the phosphor screen of a cathode ray tube.

While the invention has been described essentially with 30 relation to what is currently known as a shadow mask, it will be appreciated that it is not restricted to a mask having the specific size and pattern of perforations in such mask but is equally applicable to other types of perforate masks as well regardless of perforation pattern or size.

What is claimed is:

1. A perforate mask for assembly in a cathode ray tube to selectively transmit electron beams which comprises a perforated glass sheet having on its electron intercepting 40 surface a coating composed of a chemically active metal comprising a getter which is, in turn, covered and a protective layer of inactive metal.

2. A mask in accordance with claim 1 wherein the chemically active metal is barium and the inactive metal 45 is aluminum.

3. For use in multicolor television reception, a cathode ray tube having an electron emission source, an electron sensitive screen, and a perforate, electron-absorbing mask mounted intermediate said electron source and screen, said mask comprising a perforated sheet of glass having on its electron intercepting surface a coating composed of a chemically active metal comprising a getter which is, in turn, covered with a protective layer of inactive metal.

55 References Cited in the file of this patent

UNITED STATES PATENTS

2,437,941 Dorgelo \_\_\_\_\_ Mar. 16, 1948.  
2,777,084 Lafferty \_\_\_\_\_ Jan. 8, 1957

UNITED STATES PATENT OFFICE  
CERTIFICATE OF CORRECTION

May 12, 1959

Patent No. 2,886,730

John L. Sheldon

It is hereby certified that error appears in the printed specification of the above numbered patent requiring correction and that the said Letters Patent should read as corrected below.

Column 4, line 19, for "speak" read -- speaking --; line 41, for "covered and" read -- covered with --.

Signed and sealed this 15th day of September 1959.

(SEAL)

Attest:

KARL H. AXLINE

Attesting Officer

ROBERT C. WATSON  
Commissioner of Patents